

(No Model.)

D. BURKE.  
Water Closet Basin.

No. 233,470.

Patented Oct. 19, 1880.

Fig. 1.



Fig. 2.



Witnesses:

W. O. Gavin  
Chas. M. Higgins.

Inventor:

Dominic Burke  
by S. M. Wales & Son  
Attest.

# UNITED STATES PATENT OFFICE.

DOMINIC BURKE, OF NEW YORK, N. Y.

## WATER-CLOSET BASIN.

SPECIFICATION forming part of Letters Patent No. 233,470, dated October 19, 1880.

Application filed March 19, 1880. (No model.)

*To all whom it may concern:*

Be it known that I, DOMINIC BURKE, of New York city, State of New York, have invented certain new and useful Improvements 5 in Water-Closet Basins or Hoppers, of which the following is a specification.

My invention aims to construct basins or hoppers for water-closets in a more durable and inexpensive manner than those heretofore 10 used; and the essential feature of my invention may be stated to consist in a water-closet basin or hopper composed of hydraulic cement, which forms a new and improved article of manufacture.

15 Figure 1 of the annexed drawings presents a vertical section of a hopper constructed according to my invention. Fig. 2 gives an inverted plan view of the hollow drenching-rim of the hopper detached.

20 The hoppers or basins may be formed in any of the usual or adopted shapes or in any special shape desired, as my invention does not relate to the special form of the article. To produce the hoppers or basins according to my 25 invention, I take a good quality of hydraulic cement—preferably the quality known as “Portland” cement—and I mix the same with an equal quantity of sand in a mortar or other mixing vessel or machine, and, having prepared molds of suitable form and material to 30 shape the said hoppers or basins, I fill the same with the said cement and then allow it to set or harden in the mold, so as to form the desired shape of basin or hopper. When the 35 cement has hardened or set sufficiently I remove the casting from its mold and allow the hopper or basin thus cast to fully dry. When fully dry and hard the basins or hoppers may then be finished off by grinding or chiseling, 40 if necessary, to impart any desired degree of smoothness thereto or to correct any defects of molding, if such occur. After these operations the hoppers or basins are ready for the market and are fit to be mounted or attached 45 to the water-closets in the ordinary way, well known to plumbers, same as common crockery or iron basins or hoppers, and as thus formed they constitute a new and valuable article of trade for the described purpose. The advantages 50 of hoppers or basins made in this way are that the material as well as the mode of

manufacture is much less costly than that of the iron or crockery hoppers heretofore made, and moreover my cement hopper or basin, while possessing great strength, is proof against the 55 action of moisture, air, or alkalies to which its use exposes it, thus presenting an important advantage over iron, which rapidly deteriorates by rust, and of crockery or enamel, which is destroyed by the continued action of alkali. 60

I prefer to provide the upper edge of the basin or hopper with a hollow or grooved rim, B, through which the water is admitted to the hopper in an annular stream or series of jets, which rim is also preferably formed of hydraulic cement molded in the same manner as the body of the hopper. This rim may have a flat or beveled shoulder, e, to rest upon the edge of the hopper, and a pendent edge, d, which projects within the hopper, with a groove, 70 e, around its inner side to form an annular water-channel between the basin and the rim. The water may be admitted to this channel to flush the basin by a pipe extended through a hole, f, in the side of the basin, and it may 75 discharge into the basin through a series of dents, g, in the pendent edge of the rim. By this construction of the rim it will be observed that while the water is admitted in the required manner the pendent edge of the rim 80 rests at numerous points or intervals upon the interior of the basin and is thus well supported thereby. The rim may, however, be formed without the projecting and dented edge to bear upon the basin, and it may be supported at 85 the desired points against the interior of the basin by dabs of cement placed at frequent intervals, and this cement may be so placed as to discharge the water into the basin at any desired point, or to distribute it evenly therein, 90 as may be desired. The rim is cemented, by a suitable water-tight cement, to the basin around the top edge, so as to prevent any escape of water outward.

Instead of employing a mixture of cement 95 and sand, as is first described, I may use cement alone, or cement mixed with slag or with ground cinders, ground brick, or similar material, as will be readily understood.

Instead of making the drenching-rim of the 100 hopper as well as the body thereof of hydraulic cement, I may use a rim of crockery or metal

in connection with the cement body; but I prefer to make the rim also of cement, as described.

The basins or hoppers may be made or molded in one piece or in several pieces, afterward cemented together, according to the shape or design of the desired article.

What I claim as my invention is—

1. A water-closet basin or hopper made of hydraulic cement, or cement and sand, slag, &c., in one or more pieces, according to the

shape or design of the article required, with or without a hollow rim, substantially as herein set forth.

2. A hollow rim for water-closet basins or hoppers formed of hydraulic cement, substantially as herein shown and described.

DOMINIC BURKE.

Witnesses:

CHAS. M. HIGGINS,  
EDWARD H. WALES.